

## UNITED STATES PATENT OFFICE.

ARTHUR WINDING AND FREDERICK W. GEZELSCHAP, OF MILWAUKEE, WISCONSIN.

## BUILDING MATERIAL AND PROCESS OF MAKING SAME.

1,092,320.

Specification of Letters Patent.

Patented Apr. 7, 1914.

No Drawing.

Application filed March 28, 1910. Serial No. 551,916.

18-475

*To all whom it may concern:*

Be it known that we, ARTHUR WINDING and FREDERICK W. GEZELSCHAP, citizens of the United States, residing at Milwaukee, in the county of Milwaukee and State of Wisconsin, have invented certain new and useful Improvements in Building Material and Processes of Making the Same, of which the following is a specification.

10. This invention relates to an indurated non-metallic material, the foundation of which consists of a non-combustible substance such as asbestos, and to the process of making such material. Its object is to 15 produce a comparatively light, inexpensive and durable material for covering buildings and similar purposes, which will be practically fire and weather proof and impervious to moisture and air.
20. It consists in the peculiar method or process of producing such material and in the product of such process as hereinafter particularly described and defined in the appended claims.
25. In the production of the above mentioned material by the above mentioned method or process, asbestos or some similar incombustible or substantially incombustible substance, formed with a suitable 30 binder, such as silicate of magnesia or silicate of soda, into boards or sheets or other desired shapes, is saturated, incorporated or coated with a compound of carbon or a carbonaceous substance. This may be done 35 by subjecting the boards, sheets or other forms of asbestos or the like, to a bath or coating of coal tar or bituminous or mineral pitch heated or thinned with coal oil or other similar liquid, to make it sufficiently 40 fluid to penetrate the asbestos boards, sheets or the like, and to fill or enter the interstices therein. The material having been thus saturated or coated with coal tar or other carbonaceous compound or substance in a fluid 45 form capable when heated of depositing or forming graphitic or amorphous carbon or carbon in a substantially incombustible or refractory form, is subjected to fire or is heated to a sufficiently high temperature and 50 for a sufficient time to eliminate the volatile or combustible constituents of the carbonaceous compound or substance, leaving the asbestos or other incombustible foundation substance impregnated with the refractory

or non-inflammable residue or constituents 55 of the carbonaceous compound or substance.

By the foregoing treatment the asbestos board or the like is rendered dense, tough and durable, and is made practically impervious to moisture and air. Material so produced being light, durable and practically fire, water and weather proof, has a metallic ring, and in the various forms in which it may be made, such as boards or 60 sheets of the desired thickness and other dimensions, is admirably adapted for roofing and covering buildings and similar purposes.

As a concrete example, the process employed in the production of boards or sheets for roofing or covering buildings will be 70 specifically described.

Boards or sheets of the desired size and thickness formed in the usual way of asbestos with a suitable binder as above stated, being in a loose or porous and absorbent condition, are dipped into a bath of ordinary coal tar heated or warmed, to render it sufficiently fluid to readily and thoroughly penetrate and saturate them. They are then removed from the bath and after superfluous tar has been drained therefrom, they are placed, preferably edgewise or in an upright position, in a fire supplied with sufficient fuel to ignite the tar, which is allowed to burn till all the inflammable or combustible constituents thereof are consumed or eliminated and the fire resulting therefrom dies out. The burning of the tar produces 90 amorphous carbon, some of which adheres to the surfaces of the boards or sheets in the form of a crust or scale. Underneath this crust or scale, which serves to exclude air, graphitic carbon or carbon of crystalline 95 structure and metallic luster intimately incorporated with the asbestos, is formed by the high temperature resulting from the burning tar. The crust or scale being removed by jarring or scraping, leaves the 100 boards or sheets with smooth, dense, hard and glossy surfaces. The tar in the interior of the boards or sheets where it is not exposed directly to the flame of the fire and combustion cannot take place on account of 105 the absence of air, is highly heated and boiled or driven out to the surfaces of the boards or sheets, where it is either consumed

or converted into graphitic or amorphous carbon, leaving the interior of the boards or sheets tough, pliable and waterproof. Boards or sheets thus formed and treated are practically fire, water and weather proof, and being light, durable and somewhat flexible, are well suited for covering buildings, and similar uses.

We claim:

- 10 1. The process of making substantially water, fire and weather proof non-metallic building material, which consists in forming asbestos mixed with a suitable binder into a porous body of the desired shape and 15 dimensions, saturating such porous body with hydrocarbon having the properties of coal tar in a fluid condition, and then subjecting the saturated body to fire to ignite and burn the tar until all the inflammable 20 constituents of the hydrocarbon are eliminated and refractory carbon is formed and

burned into and intimately incorporated with the asbestos.

2. An indurated, non-metallic and substantially fire, water and weather proof 25 building material, consisting of a porous body of asbestos formed with a binder into the desired shape, impregnated with non-inflammable residue of a hydrocarbon and having a dense, hard and lustrous surface of 30 refractory carbon burned into and intimately incorporated with the asbestos and possessing tough, non-friable, pliable and water-proof characteristics.

In witness whereof we hereto affix our 35 signatures in presence of two witnesses.

ARTHUR WINDING.  
FREDERICK W. GEZELSCHAP.

Witnesses:

CHAS. L. Goss,  
ALICE E. Goss.

---